

Aug. 3, 1943.

G. F. NADEAU ET AL

2,326,057

ANTIHALATION FILM

Filed Jan. 14, 1942



Gale F. Nadeau  
Alfred D. Slack  
INVENTORS

BY *Newton M. Perrin*  
*R. Frank Smith*  
ATTORNEYS

## UNITED STATES PATENT OFFICE

2,326,057

## ANTIHALATION FILM

Gale F. Nadeau and Alfred D. Slack, Rochester, N. Y., assignors to Eastman Kodak Company, Rochester, N. Y., a corporation of New Jersey

Application January 14, 1942, Serial No. 426,738

5 Claims. (Cl. 95—9)

This invention relates to photographic film, and more particularly to photographic film protected against halation.

This invention is in part a continuation of the Nadeau and Slack U. S. Patent, 2,289,799, granted July 14, 1942 and U. S. Patent 2,311,073, granted February 16, 1943.

Antihalation coatings, for the protection of sensitive photographic film against halation, of the type removable in photographic processing solutions are well known. Antihalation coatings of the type not removable in photographic processing solutions, but which are intended to be retained, minus the antihalation dye, are less well known. Such coatings are described in the prior applications above cited.

One problem in connection with backings of the latter type after adequate measures have been taken to prevent base staining by the antihalation dyes, is to prevent the deposition of dye particles on the surface of the backing of such nature and distribution that when film is wound on a spool these particles under the influence of moisture transfer to the emulsion layer in contact therewith. This problem, not solved up to the time of the present invention, has required in many cases, the dispersion of the antihalation dye in the film support itself from which it is, of course, not removable or decolorizable with ease. Even when such desirable water-swellable coatings as those described in the prior applications cited, are used, the control of the balance between the bleachability of the dye and its tendency to bleed in water is very critical.

We have found that these defects can be eliminated by converting the dye and its carrier material to a less water-soluble salt through the use of amines slightly soluble or insoluble in water. The function of the amine is to react with the acid group of the carrier and make a less water-susceptible compound than the free acid form of the carrier. Also, the dyes, normally sulfonic acid derivatives, possess considerable water-solubility and, by their conversion to amine salts, this solubility in water is very much decreased, if not eliminated altogether. The amine salt of the dye possesses an additional advantage in that it is usually much more solvent-soluble than the free acid form of the dye.

The figure of the accompanying drawing shows in cross-sectional view a sensitive photographic film constructed in the manner of our invention. As shown therein the support 10 of a cellulose ester or other material such as a synthetic resin, is provided on one side with a sensitive emulsion

layer 11 and on the opposite side with the antihalation layer 12 of the invention, of an amine salt of a cellulose mixed organic acid ester insoluble in photographic processing solutions e. g. cellulose acetate phthalate of the composition described in the prior U. S. patent application, Serial No. 381,695, above cited, containing substantially four to eight acyl groups per C<sub>24</sub> cellulose unit, of which not more than one is a dicarboxylic acid acyl group and the remainder are aliphatic monobasic acid acyl groups of less than five carbon atoms, and an amine salt of an acid dye.

Other cellulose mixed organic acid dicarboxylic acid esters may be used, such as those containing substantially four to eight acyl groups per C<sub>24</sub> cellulose unit, of which not more than one is a dicarboxylic acid acyl group and the remainder are aliphatic monobasic acid acyl groups, e. g. cellulose valerate phthalate, caprylate succinate, etc.

The following examples typify the operation of the invention, however, they are given merely for illustration and are intended in no way to limit the scope of the invention.

## EXAMPLE 1

A photographic support such as one of cellulose acetate propionate or cellulose nitrate, suitably subbed if required as shown in Examples 1 and 4, U. S. patent application 381,694, now U. S. Patent No. 2,289,799, may be coated with a dope of the following typical composition:

|                                                           | Per cent |
|-----------------------------------------------------------|----------|
| 35 Cellulose acetate phthalate (27% acetyl, 13% phthalyl) | 4        |
| Dicyclohexylamine                                         | 1.65     |
| Aerosol AY (sodium sulfodiamyl succinate)                 | 1        |
| Acetone                                                   | 45       |
| 40 Methyl Cellosolve                                      | 20       |
| Ethyl alcohol                                             | 28.35    |

Over this layer may be applied a dye solution of the following composition:

|               | Per cent |
|---------------|----------|
| 45 "A" dye    | 1.35     |
| m-Toluidine   | 2.0      |
| Ethyl alcohol | 96.65    |

Typical dyes useful in the above formula (designated as, "A" dye, in the above formula), are fugitive dyes such as Acid Magenta (800) Acid Green (764), Acid Blue 3R (sulfonated triphenylmethane dye) and sulfonated Malachite Green (Muehler U. S. Patent No. 2,150,695, granted March 14, 1939). The numbers following the

names of the dyes refer to the Schultz Dyestuff Tables 7th edition (1931). These dyes are fugitive dyes of the acid type which readily form salts with amines and which are bleachable in photographic processing solutions. If desired, commercial amine salts of dyes such as Luxol Brilliant Green BL (guanidine salt of Acid Green) may be used in alcoholic solution for dyeing the backing layers.

EXAMPLE 2

Supports of the type described in Example 1 may be coated with an amine salt of a cellulose dicarboxylic acid ester from a solution of the following composition:

|                                                        | Per cent |
|--------------------------------------------------------|----------|
| Cellulose acetate phthalate (27% acetyl, 13% phthalyl) | 5        |
| m-Toluidine                                            | 2.5      |
| Aerosol AY                                             | 1        |
| Acetone                                                | 45       |
| Methyl Cellosolve                                      | 20       |
| Ethyl alcohol                                          | 26.5     |

Any of the following solutions may be used for dyeing this layer.

Solution A

|               | Per cent |
|---------------|----------|
| "A" dye       | 2        |
| "B" dye       | 2        |
| Diethyl amine | 2        |
| Ethyl alcohol | 94       |

Solution B

|               | Per cent |
|---------------|----------|
| "A" dye       | 1        |
| "B" dye       | 1        |
| m-Toluidine   | 2.5      |
| Ethyl alcohol | 95.5     |

Solution C

|                    | Per cent |
|--------------------|----------|
| "A" dye            | 1        |
| "B" dye            | 1        |
| 8-Hydroxyquinoline | 4        |
| Ethyl alcohol      | 94       |

The dye designated as "A" dye in solutions A, B, and C, may be a sulfonated Malachite Green dye, and "B" dye may be Acid Magenta.

In addition to the amines shown in the above formulas we may use many other organic amines such as diethyl amine, tributyl amine, diamyl amine, dicyclohexyl amine, aniline, diphenyl guanidine, etc. In choosing an amine for the purpose of our invention it should be noted that while all amines appear to be effective to a certain extent in accomplishing the objects of the invention, the amines chosen should transform the antihalation dye and carrier material to compounds possessing reduced moisture susceptibility. It is for this reason that amines possessing a minimum solubility in water are particularly useful.

It is to be understood that the disclosure herein is by way of example, and that we consider as

included in our invention all modifications and equivalents falling within the scope of the appended claims.

What we claim is:

1. A photographic film free from halation which comprises a support provided on one side thereof with a light sensitive emulsion layer, and on the opposite side with a layer containing a cellulose mixed organic acid dicarboxylic acid ester containing substantially four to eight aliphatic monobasic organic acid acyl and dicarboxylic acid acyl groups per C<sub>24</sub> cellulose unit of which not more than one is a dicarboxylic acid group and the remainder are aliphatic monobasic acid acyl groups, and a mixture of an organic amine and an acid dye.

2. A photographic film free from halation which comprises a support provided on one side thereof with a light sensitive emulsion layer, and on the opposite side with a layer containing an amine salt of a cellulose mixed organic acid dicarboxylic acid ester containing substantially four to eight aliphatic monobasic organic acid acyl and dicarboxylic acid acyl groups per C<sub>24</sub> cellulose unit of which not more than one is a dicarboxylic acid group and the remainder are aliphatic monobasic acid acyl groups, and an amine salt of an acid dye.

3. A photographic film free from halation which comprises a support provided on one side thereof with a light sensitive emulsion layer, and on the opposite side with a layer containing a cellulose mixed organic acid dicarboxylic acid ester containing substantially four aliphatic monobasic organic acid acyl and dicarboxylic acid acyl groups per C<sub>24</sub> cellulose unit of which not more than one is a dicarboxylic acid acyl group and the remainder are aliphatic monobasic acid acyl groups, and an amine salt of an acid dye.

4. A photographic film free from halation which comprises a support provided on one side thereof with a light sensitive emulsion layer, and on the opposite side with a layer containing an amine salt of a cellulose mixed organic acid dicarboxylic acid ester containing substantially eight aliphatic monobasic organic acid acyl and dicarboxylic acid acyl groups per C<sub>24</sub> cellulose unit of which not more than one is a dicarboxylic acid acyl group and the remainder are aliphatic monobasic acid acyl groups, and an amine salt of an acid dye.

5. A photographic film free from halation which comprises a support provided on one side thereof with a light sensitive emulsion layer, and on the opposite side with a layer containing an amine salt of a cellulose mixed organic acid dicarboxylic acid ester containing substantially four to eight acyl groups per C<sub>24</sub> cellulose unit of which one is a dicarboxylic acid acyl group and the remainder are aliphatic monobasic acid acyl groups, and an amine salt of an acid dye.

GALE F. NADEAU.  
ALFRED D. SLACK.